

## UNITED STATES PATENT OFFICE.

JAMES BADDILEY, PERCY CHORLEY, AND CARLTON BUTLER, OF MANCHESTER, ENGLAND, ASSIGNORS TO BRITISH DYESTUFFS CORPORATION LIMITED, OF MANCHESTER, ENGLAND.

## PROCESS OF DYEING ARTIFICIAL SILK.

No Drawing. Application filed April 2, 1927, Serial No. 180,611, and in Great Britain June 7, 1926.

This invention relates to dyeing and is an improvement in or a modification of the invention described in our copending application No. 180,610, filed April 2, 1927, according to which we have discovered that the secondary disazo dyestuffs obtained by coupling aminosalicylic acids or their homologues, hereafter referred to as amino-o-hydroxy-carboxy acids of the benzene series, with the usual middle components, further diazotizing and combining with the peri-substituted naphthalene sulpho acids as end-components, have a good affinity for regenerated cellulose silks and possess the valuable property of giving level dyeings on these fibres.

We have now found that in addition to the said disubstituted naphthalene sulpho acid components used in our previous application there may be used as end components coupling components of the naphthalene series containing a single auxochromic group, namely naphthols, naphthylamines and their N-substitution products, and sulphonated derivatives of these classes. The present invention consists in the dyeing of regenerated silks, such as viscose silk, with the secondary disazo dyestuff obtained by combining amino-o-hydroxy-carboxy acids of the benzene series with the usual middle components, further diazotizing and combining with a coupling of the naphthalene series, namely a naphthol, or a naphthylamine or an N-substitution product of the latter, or with a sulphonated derivative of one of these. As middle components there may be used  $\alpha$ -naphthylamine, 1-amino-2-naphthol ethers, 1-naphthylamine-6- or 7-sulphonic acids, 1-amino-2-alkoxy-naphthalene-6- or 7-sulphonic acids, meta-amino-para-cresol methyl ether, amino-hydroquinone-dimethyl ether and the like.

The dyestuffs so obtained have a wide range of shades according to the end component chosen, and they give level dyeings on regenerated cellulose silks. Some of these dyestuffs are already known and have been used for dyeing wool, particularly for producing blacks by after-treatment with chromium compounds, but it was not foreseen that they would have a good affinity for regenerated cellulose silks and that they would give level dyeings on these fibres.

The fibres are dyed in the usual way, the

following description being typical, but we do not limit ourselves to the conditions quoted (the parts are by weight):—

The dyebath is made up from 3000 parts of water, 20 parts of Glauber's salt, 2 parts of soap and one part of solochrome black F (Colour Index No. 299). 100 parts of the regenerated cellulose silk are entered into the bath at about 30° C. The bath is then heated to about 90° C. and dyeing allowed to proceed for about one hour. The silk is then removed, rinsed and dried. The resulting dyeing is a level deep black shade. By after-treating the dyed fabric with chromium fluoride the fastness to washing is considerably increased.

Other examples to illustrate our invention are quoted in the following table:—

| Secondary disazo dyestuff from—          |                                          |                                             | Shade on viscose silk | 75  |
|------------------------------------------|------------------------------------------|---------------------------------------------|-----------------------|-----|
| First component                          | Middle component                         | End component                               |                       |     |
| 5-aminosalicylic acid.                   | $\alpha$ -naphthylamine.                 | 1-naphthol-4-sulphonic acid.                | Black.                |     |
| Ditto.                                   | ditto.                                   | 1-naphthol-5-sulphonic acid.                | Violet black.         |     |
| Ditto.                                   | ditto.                                   | 2-naphthylamine-6-sulphonic acid.           | Bordeaux.             | 80  |
| Ditto.                                   | ditto.                                   | 2-methylamine-naphthalene-7-sulphonic acid. | Violet.               |     |
| Ditto.                                   | ditto.                                   | 1-phenylamino-naphthalene-8-sulphonic acid. | Brown.                |     |
| Aminosalicylic acid (technical mixture). | ditto.                                   | 2-naphthol-6-sulphonic acid.                | Blue-violet.          | 85  |
| Ditto.                                   | ditto.                                   | 1-naphthylamine-4-sulphonic acid.           | Brownish violet.      |     |
| Ditto.                                   | ditto.                                   | 1-naphthylamine-6 and 7-sulphonic acids.    | Violet brown.         | 90  |
| Ditto.                                   | 1-naphthylamine-6 and 7-sulphonic acids. | 1-naphthol-4-sulphonic acid.                | Violet.               |     |
| Ditto.                                   | ditto.                                   | 1-naphthol-5-sulphonic acid.                | Ditto.                |     |
| Ditto.                                   | ditto.                                   | 1-naphthol-3,6-disulphonic acid.            | Bluish-violet.        | 95  |
| Ditto.                                   | ditto.                                   | Ethyl- $\alpha$ -naphthylamine.             | Violet.               |     |
| Ditto.                                   | ditto.                                   | $\beta$ -naphthol.                          | Red-violet.           |     |
| Ditto.                                   | ditto.                                   | $\alpha$ -naphthylamine.                    | Violet.               |     |
| Ditto.                                   | $\alpha$ -naphthylamine.                 | ditto.                                      | Chocolate.            |     |
| Ditto.                                   | $\beta$ -xylydine.                       | 2-naphthol-6-sulphonic acid.                | Red-violet.           |     |
| Ditto.                                   | 1-amino-2-naphthol ethyl ether.          | 2-naphthol-7-sulphonic acid.                | Greenish-blue.        | 100 |

What we claim and desire to secure by Letters Patent is:—

1. The dyeing process which comprises dyeing regenerated cellulose silks with secondary disazo dyestuffs made by combining

amino-o-hydroxy-carboxy-acids of the benzene series with the usual middle components, further diazotizing and combining with a coupling component of the naphthalene series containing a single auxochromic group.

2. The dyeing process which comprises dyeing regenerated cellulose silks with the secondary disazo dyestuffs made by combining an amino salicylic acid with the usual middle components, further diazotizing and combining with a coupling component of the naphthalene series containing a single auxochromic group.

15 3. The dyeing process which comprises

dyeing regenerated cellulose silks with the secondary disazo dyestuffs made by combining 5-amino-salicylic acid with the usual middle components, further diazotizing and combining with a coupling component of the naphthalene series containing a single auxochromic group.

4. As new industrial products, regenerated cellulose silks when dyed by the process claimed in claim 1.

25

In testimony whereof we affix our signatures.

JAMES BADDILEY.  
PERCY CHORLEY.  
CARLTON BUTLER.